

## UNITED STATES PATENT OFFICE

2,289,367

## PHOTOGRAPHIC DEVELOPER

John David Kendall, Ilford, England, assignor to  
Ilford Limited, Ilford, England, a British company

No Drawing. Application May 28, 1941, Serial  
No. 395,680. In Great Britain July 10, 1940

13 Claims. (Cl. 95—88)

This invention relates to photographic development processes and in particular to the development of latent images formed in silver halide photographic emulsions.

It is an object of this invention to provide a new series of compounds capable of acting as photographic developers. It is a further object of this invention to provide new photographic developing compositions. A still further object of the invention is to provide a substitute for Metol (1-methyl-amino-4-hydroxy benzene) in photographic developers. Other objects will appear hereinafter.

According to this invention the development of latent images formed in photographic materials bearing silver halide emulsions is effected by treating the materials with a solution containing a 3-pyrazolidone of the general formula:



where R<sub>1</sub>, R<sub>2</sub> and R<sub>3</sub> are the same or different and are hydrogen atoms or hydrocarbon groups, for instance, alkyl groups, e. g. methyl, ethyl, propyl, isopropyl or higher alkyl groups, aryl groups, e. g. phenyl and naphthyl groups or aralkyl groups, e. g. benzyl groups. Such hydrocarbon substituent groups may themselves be substituted; for example, aryl groups may be substituted with hydroxy, alkoxy, oxyalkyl, amino, substituted amino, nitro, sulphonic or carboxylic groups or halogen atoms.

Specific 3-pyrazolidones which may be employed according to this invention are 3-pyrazolidone itself, 5-phenyl-3-pyrazolidone, 1-phenyl-3-pyrazolidone, 1-phenyl-5-methyl-3-pyrazolidone and 1-p-chlorophenyl-3-pyrazolidone. Compounds in which the group R<sub>1</sub> in the above formula is an aryl group, and the groups R<sub>2</sub> and R<sub>3</sub> are hydrogen atoms are especially valuable developing agents according to this invention.

The 3-pyrazolidones may be prepared by var-

ious methods. Thus compounds in which R<sub>1</sub> in the above general formula is an hydrogen atom may be prepared by condensing hydrazine hydrate with an  $\alpha$ - $\beta$ -olefine carboxylic acid of the general formula:



Compounds in which R<sub>1</sub> is a hydrocarbon group 10 may be prepared by condensing the corresponding hydrocarbon-substituted hydrazine with a  $\beta$ -halogen-substituted fatty acid of the general formula:



X being a halogen atom, e. g. chlorine, bromine or iodine.

The developing agents of this invention may 20 be employed in developing compositions in which they form the sole active developing agents or they may be employed in developing compositions which also contain other active developing agents. A particularly valuable developing 25 agent according to this invention is 1-phenyl-3-pyrazolidone. This compound has developing qualities which somewhat resemble those of metol (1-methyl-amino-4-hydroxy-benzene sulphate). It has a very low inertia period i. e. 30 development sets in very rapidly, and it yields developed images of soft contrast. It may be satisfactorily used as a substitute for metol in all types of developing compositions in which metol has hitherto been employed. However, 35 it presents the very distinct advantage over metol that, used as a substitute for metol in developing solutions containing other developers in addition to the metol, e. g. hydroquinone or pyrogallic acid, it may be employed in concentrations much smaller than those in which metol is normally employed, whilst retaining similar developing properties.

Thus, for example, replacement of the metol 45 in a metol-hydroquinone developer by about  $\frac{1}{15}$  to  $\frac{1}{6}$  of its weight of 1-phenyl-3-pyrazolidone according to the particular developer composition yields a developer of similar development characteristics to the initial metol-hydroquinone developer.

The compounds of this invention may also be

employed as substitutes for part only of the metol in metol-type developers, and in general the compounds may be employed as additions to all types of developer compositions where they serve as agents to decrease the inertia period of such developing compositions.

The following examples illustrate the invention:

#### EXAMPLE I

In this example 1-phenyl-3-pyrazolidone is employed as the sole developing agent.

#### Developer

|                                |       |     |
|--------------------------------|-------|-----|
| 1-phenyl-3-pyrazolidone        | grams | 3   |
| Sodium sulphite (crystalline)  | do    | 25  |
| Sodium carbonate (crystalline) | do    | 50  |
| Potassium bromide              | do    | 0.5 |
| Water to make up to            | ccs   | 500 |

For use, one part of this developer is diluted with three parts of water. It is a very soft-working developer giving results of a similar character to those obtained from a similar developer containing an equal weight of metol as the sole developing agent, but of softer contrast.

#### EXAMPLE II

In this example 1-phenyl-3-pyrazolidone is used as a substitute for the metol in a metol-hydroquinone developer.

#### Developer

|                                |       |      |
|--------------------------------|-------|------|
| 1-phenyl-3-pyrazolidone        | grams | 0.15 |
| Sodium sulphite (crystalline)  | do    | 75   |
| Hydroquinone                   | do    | 4    |
| Sodium carbonate (crystalline) | do    | 50   |
| Potassium bromide              | do    | 1    |
| Water to make up to            | ccs   | 500  |

For use, one part of this developer is diluted with two parts of water. It yields results which are very closely similar to those obtained from a similar developer containing 1 gram of metol instead of the 0.15 gram of 1-phenyl-3-pyrazolidone. Thus it will be noted that by substituting for the metol in this standard type of metol-hydroquinone developer,  $\frac{1}{4}$  of its weight of 1-phenyl-3-pyrazolidone, a developer of very similar characteristics is obtained.

#### EXAMPLE III

In this example, 1-phenyl-3-pyrazolidone is used as a substitute for the metol in a metol-pyrogallic acid type of developer.

#### Developer

##### Solution A:

|                          |       |     |
|--------------------------|-------|-----|
| 1-phenyl-3-pyrazolidone  | grams | 0.2 |
| Potassium metabisulphite | do    | 6   |
| Pyrogallic acid          | do    | 6   |
| Water to make up to      | ccs   | 500 |

##### Solution B:

|                                |       |     |
|--------------------------------|-------|-----|
| Sodium carbonate (crystalline) | grams | 100 |
| Water to make up to            | ccs   | 500 |

For use, equal parts of solutions A and B are mixed together. The developer has properties very closely similar to those obtained from a corresponding developer containing 2 grams of metol instead of the 1-phenyl-3-pyrazolidone. In other words, by substituting for the metol in this standard type of developer, only  $\frac{1}{4}$  of its weight of 1-phenyl-3-pyrazolidone, a developer of very similar characteristics is obtained.

#### EXAMPLE IV

This illustrates the addition of 1-phenyl-3-pyrazolidone to a metol hydroquinone developer.

5

#### Developer

|                                  |       |     |
|----------------------------------|-------|-----|
| 1-phenyl-3-pyrazolidone          | grams | 1.0 |
| Metol                            | do    | 1.0 |
| 10 Sodium sulphite (crystalline) | do    | 75  |
| Hydroquinone                     | do    | 4   |
| Sodium carbonate (crystalline)   | do    | 50  |
| Potassium-bromide                | do    | 1   |
| Water to make up to              | ccs   | 500 |

15

For use, one part of this developer is diluted with 2 parts of water.

20

This developer is much more rapid in action than a developer not containing the 1-phenyl-3-pyrazolidone but otherwise of the same composition. The increase in the speed of development due to the presence of the 1-phenyl-3-pyrazolidone in the above developer compositions is shown by the following figures which were obtained on development of a fast panchromatic emulsion.

|    | Development time at 65° F. | Gamma values                                |                                                 |
|----|----------------------------|---------------------------------------------|-------------------------------------------------|
|    |                            | Developer including 1-phenyl-3-pyrazolidone | Developer not including 1-phenyl-3-pyrazolidone |
| 30 | 2 minutes                  | 1.13                                        | 0.64                                            |
| 35 | 4 minutes                  | 1.42                                        | 1.06                                            |

Thus it will be seen that the developer containing 1-phenyl-3-pyrazolidone gives an image of slightly higher contrast in two minutes' development than is obtained in four minutes without the 1-phenyl-3-pyrazolidone.

The foregoing examples are intended primarily to shew the variability of application of the developers and they all specify the compound 1-phenyl-3-pyrazolidone. It is to be understood however, that any other 3-pyrazolidone included within the scope of this invention may be similarly employed. Thus, equal weight of 1-p-tolyl-3-pyrazolidone, 1-p-chlorphenyl-3-pyrazolidone, and 1-phenyl-5-methyl-3-pyrazolidone substituted for the 1-phenyl-3-pyrazolidone of Example II above give developers of very similar characteristics, the developed images obtained in the case of developers containing 1-p-chlorphenyl-3-pyrazolidone and 1-phenyl-5-methyl-3-pyrazolidone being of somewhat softer contrast.

#### What I claim is:

1. A photographic developing composition containing a 3-pyrazolidone of the general formula:



where R1, R2 and R3 are selected from the class consisting of hydrogen atoms and hydrocarbon groups.

2. A photographic developing composition con-

taining hydroquinone and a 3-pyrazolidone of the general formula:



where R<sub>1</sub>, R<sub>2</sub> and R<sub>3</sub> are selected from the class consisting of hydrogen atoms and hydrocarbon groups.

3. A photographic developing composition containing pyrogallic acid and a 3-pyrazolidone of the general formula:



where R<sub>1</sub>, R<sub>2</sub> and R<sub>3</sub> are selected from the class consisting of hydrogen atoms and hydrocarbon groups.

4. A photographic developing composition containing 1-methylamino-4-hydroxy benzene, hydroquinone and a 3-pyrazolidone of the general formula:



where R<sub>1</sub>, R<sub>2</sub> and R<sub>3</sub> are selected from the class consisting of hydrogen atoms and hydrocarbon groups.

5. A photographic developing composition containing 1-phenyl-3-pyrazolidone.

6. A photographic developing composition containing 1-phenyl-3-pyrazolidone and hydro-

7. A photographic developing composition containing 1-phenyl-3-pyrazolidone and pyrogallic acid.

8. A photographic developing composition containing 1-phenyl-3-pyrazolidone, 1-methylamino-4-hydroxy benzene and hydroquinone.

9. An alkaline photographic developing composition containing an alkali metal sulfite, an alkali metal carbonate and a 3-pyrazolidone of the general formula:



20 where R<sub>1</sub>, R<sub>2</sub> and R<sub>3</sub> are selected from the class consisting of hydrogen atoms and hydrocarbon groups.

10. An alkaline photographic developing composition containing an alkali metal sulfite, an alkali metal carbonate, potassium bromide, and a 3-pyrazolidone of the general formula:



30 where R<sub>1</sub>, R<sub>2</sub> and R<sub>3</sub> are selected from the class consisting of hydrogen atoms and hydrocarbon groups.

40 11. A photographic developing composition containing an alkali metal sulfite, an alkali metal carbonate, and 1-phenyl-3-pyrazolidone.

12. A photographic developing composition containing an alkali metal sulfite, an alkali metal carbonate, and 1-phenyl-3-pyrazolidone and pyrogallic acid.

13. A photographic developing composition containing an alkali metal sulfite, an alkali metal carbonate, and 1-phenyl-3-pyrazolidone, 1-methylamino-4-hydroxy benzene and hydroquinone.

JOHN DAVID KENDALL.